

## 1

3,074,386

## DIESEL FUEL OIL

Raymond Gay, Notre-Dame-de-Gravenchon, and Emmanuel Siganos, Lavera, France, assignors to Esso Research and Engineering Company, Elizabeth, N.J., a corporation of Delaware  
 No Drawing. Filed Mar. 7, 1960, Ser. No. 12,919  
 Claims priority, application France Mar. 17, 1959  
 8 Claims. (Cl. 123—1)

The present application relates to fuel oils having improved combustion efficiency.

The term "fuel oil" in general comprises all liquid hydrocarbons used as fuels for burners and furnaces and the like, or as fuels for diesel engines, and includes both residual oils and distillate oils such as gas oil. The fuel oil may, for example, have a Luchaire flash point above 60° C.

It is generally necessary to improve the properties, in particular the combustion efficiency, of fuel oils. It has been observed, particularly in diesel engines, that when the quantity of fuel injected is increased, smoke, increasing with the quantity of fuel injected, appears in the exhaust gases. This is due to the incomplete combustion of the fuel which decreases the combustion efficiency of the engine and also causes engine fouling.

It has now been discovered that fuel oils of improved combustion efficiency are obtained when the fuel oil contains a minor proportion of an oil-soluble compound formed by reacting an organic base, or an alkylene oxide containing from 2 to 6 carbon atoms, with an organic derivative of phosphoric acid having the general formula:



wherein X represents oxygen or sulphur, R' and R'' represent alkyl or substituted alkyl radicals containing from 2 to 20 carbon atoms, preferably 8 to 14 carbon atoms.

The oil-soluble organic phosphorus compounds of the present invention are self-dispersing in fuel oils and are derivatives of phosphoric acid in which an acid hydrogen is combined with:

(1) An organic base such as an amine to form a salt of formula:



in which X represents oxygen or sulphur, R'' and R' may be alkyl radicals having for preference from 2 to 20 atoms, better still 8 to 14 atoms of carbon. These radicals may or may not have substituent groups such as OH, NH<sub>2</sub>, SH, CN etc.; R''' may be an alkyl radical having for preference from 4 to 18 and better still from 6 to 12 carbon atoms.

(2) An alkylene oxide having for preference from 2 to 6 carbon atoms, to yield in the case of ethylene oxide the derivatives complying with the general formula:



in which X, R' and R'' have the same meaning as in the previous formula and n represents a whole number.

According to the invention, the amines used may be of the straight or branched chain type, primary or secondary, mono-amines or polyamines, amido-amines or ethanolamines.

The quantity of organic derivative of phosphoric acid to be added to the fuel oil is for the preference between

## 2

0.005 and 5% better still between 0.05 and 1% by weight in relation to the fuel oil.

This organic derivative of phosphoric acid is particularly suitable for improving gas oils, domestic fuel oils, light and heavy fuel oils, i.e. light hydrocarbons having a Luchaire flash point above 60° C.

The following examples given by way of explanation will better show the scope and importance of the invention.

10 The tests were carried out with a diesel engine of General Motors (GM 371) possessing the following characteristics:

Number of cylinders ..... 3.  
 15 Bore in mm. ..... 108 (4 1/4 inches).  
 Stroke in mm. ..... 127 (5 "inches").  
 Cylinder capacity in cc. ..... 3474 (212 cubic inches).  
 Temperature of water ..... 80° C.  
 Temperature of oil ..... 107° C.  
 20 Speed ..... 1200 r.p.m.

Smoke measurements at the exhaust have been carried out by means of the smoke meter known by the name of the "Von Brand Smoke-meter." This apparatus makes it possible to effect the measurement of the smoke contained in the exhaust gases, by causing the latter to pass through a paper screen unwinding at constant rate. The intensity of the spot is obtained by interpolation between two standards (one white and the other black), by measuring the percentage of light reflected with the aid of a photo-reflecto-meter.

25 By running the diesel engine with a determined output and feeding it with a gas oil with or without additive, the following characteristics were measured,

30 I=smoke index (100 corresponds to the black band) as percent reflectance

C=consumption in litres/hour

t=mean temperature of the exhaust gases in ° C.

and the following calculation was made:

40 Consumption of gas oil with additive  

$$\Delta C = \frac{\text{consumption gas oil without additive}}{\text{Consumption of fuel oil without additive}} \times 100$$

## EXAMPLE I

With the use of a gas oil having the following characteristics:

45 Density at 15° C. ..... 0.857  
 Engler viscosity at 20° C. ..... 1.43  
 Sulphur ..... 1%  
 Cetane number ..... 48

50 the following results were obtained, using as additive according to the invention the product resulting from the neutralization of dilaurophosphoric acid with octylamine in the proportion of 0.6 g. per kg. of gas oil.

Table I

| 60 |                      | Output in H.P. |       |       |       |       |       |       |
|----|----------------------|----------------|-------|-------|-------|-------|-------|-------|
|    |                      | 39             | 42    | 45    | 48    | 51    | 54    | 55.8  |
| 65 | Datum Gas Oil:       |                |       |       |       |       |       |       |
|    | I                    | 13.5           | 15.5  | 16.5  | 19.5  | 24.5  | 28.5  | 34.5  |
|    | C                    | 9.56           | 10.28 | 11.01 | 11.89 | 12.53 | 12.98 | 13.57 |
|    | t, ° C               | 238            | 253   | 267   | 282   | 297   | 309   | 321   |
| 70 | Gas Oil + additives: |                |       |       |       |       |       |       |
|    | I                    | 7.5            | 9.5   | 11.5  | 14.5  | 20.5  | 24.5  | 31.5  |
|    | C                    | 9.44           | 10.17 | 10.86 | 11.59 | 12.44 | 12.87 | 13.53 |
|    | ΔC                   | -1.22          | 1.04  | -1.30 | -0.85 | -0.68 | -0.83 | -0.25 |
|    | t, ° C               | 236            | 250   | 264   | 280   | 296   | 305   | 318   |

These results show that the application of the additive according to the invention makes it possible to:

- (1) Obtain less smoke for a given output.
- (2) Obtain more power for a given smoke index.
- (3) Lessen consumption.

#### EXAMPLE II

Using the same gas-oil as in Example I, the following results were obtained, using as additive according to the invention ethoxy-dilaurophosphoric acid with 6 molecules of ethylene oxide in the proportion of 0.6 g. per kg. gas oil.

Table II

|                            | Output in H.P. |    |    |    |    |
|----------------------------|----------------|----|----|----|----|
|                            | 42             | 45 | 48 | 51 | 54 |
| Datum Gas-Oil: L.....      | 10             | 13 | 19 | 25 | 33 |
| Gas-oil + additive: L..... | 8              | 10 | 17 | 23 | 32 |

It is obvious that this invention has only been described by way of explanation and in no sense restrictively.

What is claimed is:

1. An improved diesel fuel oil composition containing between 0.005 and 5.0 weight percent of an oil soluble organic phosphorus additive having the formula:



wherein X is selected from the group of oxygen and sulfur, R' and R'' are alkyl radicals of from 2 to 20 carbon atoms, and n is a whole number from 2 to 6, said compound enhancing the combustion efficiency of said diesel oil.

2. A diesel fuel oil composition as defined in claim 1 wherein said oil soluble additive is added in an amount between 0.05 and 1.0 weight percent.

3. A diesel fuel oil composition as defined in claim 1 wherein said X is oxygen, R' and R'' have from 8 to 14 carbon atoms, and n is 6.

4. A diesel fuel oil composition as defined in claim 1 wherein said diesel oil has a Luchaire flash point above 60° C.

5. A process of operating a diesel engine, which process comprises adding to a diesel fuel oil between 0.005 and 5.0 weight percent of an oil soluble organic phosphorus additive having the formula:



10 15 wherein X is selected from the group of oxygen and sulfur, R' and R'' are alkyl radicals of from 2 to 20 carbon atoms, and n is a whole number from 2 to 6, and combusting said fuel in said engine, thereby enhancing the combustion efficiency and reducing the tendency of said engine to smoke.

20 25 6. A process as defined by claim 5 wherein said oil soluble additive is added in an amount between 0.05 and 1.0 weight percent.

7. A process as defined by claim 5 wherein said X is oxygen, R' and R'' have from 8 to 14 carbon atoms, and n is 6.

25 30 8. A process as defined by claim 5 wherein said fuel oil is a diesel oil having a Luchaire flash point above 60° C.

#### References Cited in the file of this patent

#### UNITED STATES PATENTS

|           |                        |                |
|-----------|------------------------|----------------|
| 2,335,953 | McCracken et al. ----- | Dec. 7, 1943   |
| 2,602,049 | Smith et al. -----     | July 1, 1952   |
| 2,793,945 | Walker et al. -----    | May 28, 1957   |
| 2,841,126 | Cantrell et al. -----  | July 1, 1958   |
| 2,905,542 | Gottshall et al. ----- | Sept. 22, 1959 |
| 2,979,523 | Cantrell et al. -----  | Apr. 11, 1961  |